

# UNITED STATES PATENT OFFICE.

AUGUSTE EDWARD CHARBONNEAUX, OF LOS ANGELES, CALIFORNIA.

## EXPLOSIVE.

No. 886,038.

Specification of Letters Patent. Patented April 28, 1908.

Application filed October 1, 1907. Serial No. 395,392.

*To all whom it may concern:*

Be it known that I, AUGUSTE EDWARD CHARBONNEAUX, a citizen of France, residing at Los Angeles, in the county of Los Angeles, 5 State of California, have invented a new and useful Composition of Matter Entitled Explosive, of which the following is a specification.

My composition consists of the following 10 ingredients mixed in the proportion stated, viz:—

Saccharin,  $C_6H_4SO_2CO.NH$ , 1 part by weight, Potassium chlorate,  $KClO_3$ , 3 parts by weight.

15 To obtain a quick firing explosive these ingredients are first finely powdered and then intimately mixed in a mortar. The velocity of firing or explosion depends upon the fineness to which the ingredients are powdered, a mixture of coarse crystals making a slow firing explosive. The mixture may also be very finely powdered and formed into a paste to be subsequently pressed or otherwise molded into large cubes or other shapes 20 so as to form a very slow firing explosive for use in firearms, large guns and the like.

The above mixture forms an explosive of high efficiency and great explosive energy, and is therefore well suited to the needs of 30 modern ordnance. A typical equation of the explosion of this powder is as follows:—



35 The atomic weight of saccharin being about 183 and that of potassium chlorate 122,

the proportions of the above equation are correct for the proportion of one to three by weight.

The above equation may be taken as typical of the reactions consummated during the firing of the explosive but other minor reactions may take place due to the presence of foreign substances in proximity to the explosive or due to the oxygen in the surrounding air. It will be noted from the above 40 equation that all the resultant compounds are gases with the exception of the potassium chlorid and it is immediately due to this fact that my explosive is of such high efficiency.

This explosive will not fire by means of a 50 mere blow, unless violent, but must be fired by a fuse or a cap which will transmit a flame to the mass.

Having thus described my invention what I claim as new and desire to secure by Letters 55 Patent is:—

1. The herein described composition of matter for an explosive consisting of saccharin and potassium chlorate.

2. The herein described composition of 60 matter for an explosive consisting of saccharin one part by weight and potassium chlorate three parts by weight.

In witness that I claim the foregoing I have hereunto subscribed my name this 24th 65 day of September, 1907.

AUGUSTE EDWARD CHARBONNEAUX.

Witnesses:

IRWIN H. BARBELEW,  
OLIE PALMER.